

# UNITED STATES PATENT OFFICE.

HENRY DREYFUS, OF BASEL, SWITZERLAND.

## SUBSTITUTE FOR CELLULOID AND METHOD OF MAKING SAME.

1,181,859.

Specification of Letters Patent.

Patented May 2, 1916.

No Drawing.

Application filed October 2, 1911. Serial No. 652,445.

To all whom it may concern:

Be it known that I, HENRY DREYFUS, doctor of philosophy, chemist, a citizen of the Republic of Switzerland, residing at Basel, Switzerland, (whose post-office address is 69 Schützenmattstrasse, Basel, Switzerland,) have invented a Substitute for Celluloid and Method of Making Same, of which the following description is a specification.

10 Heretofore I have applied for patents in the following countries: In France on the 15th July 1911; in Germany the 17th July 1911.

15 My invention relates to the manufacture of non-flammable and inflammable celluloids or of solutions of cellulosic esters and of products and objects of all kinds dependent thereon.

20 The object of my invention is to provide a new and improved process and new products.

In the present invention a whole series of products have been found which are capable of replacing camphor with great advantage. These products can be employed both 25 with cellulose acetates or cellulose esters of other fatty acids; they can be used with the same advantage with mixtures of nitro-cellulose and acetate of cellulose or other cellulosic esters. If cellulose acetates or other 30 analogous cellulosic esters are exclusively employed in combination with these new camphor substitutes, the resulting products are comparatively non-inflammable.

35 The solvents or camphor substitutes employed in the present invention are the following:

(A) The ethers of phenols, cresols, and their homologues, for example: anisol,



40 phenetol



(B) The ethers of naphthols, such as those of alpha- or beta-naphthol, such as methyl 45 or ethyl ethers, or homologues thereof.

(C) Ethers of poly-hydric phenols, such as those of resorcinol, pyrocatechol, such as the methyl or ethyl ethers, or homologues thereof, for example: veratrol,

50  $\text{CH}_3-\text{O}-\text{C}_6\text{H}_4-\text{O}-\text{CH}_3$

pyrocatechol diethyl ether



55 (D) Ethers of higher aromatic alcohols

such as those of benzyl alcohol, for example benzyl methyl ether



(E) Other etherified derivatives such as 60 saffrol,



isosafrol,



65

(F) Ethers of phenols (or the like as above stated) which have been etherified with phenols (or the like as above stated), 70 such as diphenyl ether,



(G) Mixtures of two or more of the materials referred to in the above paragraphs 75 A to F. With these new products it is possible, according to desire or requirement, to manufacture hard or soft materials in any gradation, employing them alone or adding oils such as castor oil or any other additions 80 or filling substances. These products are indifferent toward organic or inorganic coloring matters and the usual filling substances, and they mix with these latter in a manner analogous to that practised with ordinary celluloid made with camphor.

85 These substances are characterized by their great stability, being at least as stable as camphor. Camphor, when used in conjunction with nitrocellulose exerts no other action than its solvent action. It does not decompose, form acids, etc., and accordingly does not have any bad effects on the nitrocellulose, and in the same way neither do the substances which I use in my process, and the substances I use have the advantages over camphor that they do not burn, and are not as volatile as camphor. These products are also very stable, that is, at least as stable as camphor, and many are more stable. 100 These products may be, for the most part, prepared in a comparatively pure state at the cost much less than that of camphor.

105 The products or series of products may be employed alone or in mixtures of two or more together, and preferably in presence of alcohol or substitutes thereof or of mixtures of such substitutes with or without alcohol. These products may also be employed simultaneously and in combination with those 110

indicated in my copending application, 652,444, filed concurrently herewith, that is to say with the chlorinated derivatives of ethylene and ethane, such as dichlorethylene, 5 pentachlorethane, tetrachlorethane, trichloroethylene, or their mixtures.

If the proportions of the quantities employed are suitably chosen, the resulting materials can be worked up on the usual celluloid machines, for example rollers, presses, etc., as well as cast directly to make objects of any shape and kind according to particular desires or requirements. These products may also be employed alone or in combination 10 with the chlorinated derivatives of ethylene or ethane, for the manufacture of solutions of any nature and for any other use whatever, such as for the manufacture of varnishes, lacquers, films, artificial silk, 15 artificial horse hair, coatings of all kinds, etc., and for other employments. It has moreover been found that these products can also be employed in combination with bodies such as ethylene chlorid, methylene 20 chlorid, ethylidene chlorid, methylal and its homologues, either singly or mixed, and also in combination with the chlorinated derivatives of ethylene and ethane and particularly 25 in presence of alcohol or substitutes therefor or of mixtures of such substitutes with or without alcohol. The products above mentioned, such for example as ethylene chlorid, methylene chlorid, ethylidene chlorid, methylal and its homologues, at the 30 same time represent a series of new solvents for the acetates of cellulose; thus for example ethylidene chlorid represents a very advantageous substitute for chloroform and tetrachlorethane, and like these latter 35 dissolves the acetates or other cellulosic esters that are soluble in chloroform, while the cellulosic esters that are difficultly soluble or insoluble in chloroform are likewise insoluble in this product, but certain of said esters give concentrated and viscous solutions 40 therein on addition of alcohol. The other chlorinated derivatives such as methylene chlorid, etc., behave in the same way.

Now I have found in the course of the 45 present invention that especially the acetates of cellulose that are readily soluble in mixtures of alcohol and tetrachlorethane, are capable on heating with a mixture of trichlorethylene and alcohol, of giving viscous and concentrated solutions which congeal 50 on cooling; it is advantageous to employ mixtures of alcohol and trichlorethylene in proportions of equal volumes; if one adds to these solutions other solvents such for example as dichlorethylene, pentachloroethane, manol (methyl acetanilid tetrachlorethane, anisol, dichlorbenzenes, etc., the solutions remain liquid even on cooling.

The solvents of low boiling point, such as

dichlorethylene, trichlorethylene, ethylene 65 chlorid, methylene chlorid, ethylidene chlorid, etc., may be employed alone or in mixtures of two or more together, and in presence of alcohol or alcohol substitutes or of mixtures of such substitutes with or without 70 alcohol. The employment of these latter products in many cases presents an advantage over products having a higher boiling point, such as tetrachlorethane, anisol, etc., or their mixtures, and especially so in 75 cases where it is desired to obtain easy and rapid evaporation. Thus one preferably employs for example a quarter to half a kilo or more of these products to a kilo of acetylated cellulose, according to the particular 80 employment in view, and half a liter to a liter or more of alcohol. The alcohol may be replaced by its substitutes or as before mentioned by mixtures of such substitutes with or without alcohol. Some of these 85 products may be employed without alcohol or alcohol substitutes.

The procedure for the preparation of solutions with solvents of low boiling points, such as the alcohols and chlorinated compounds above referred to, together with the herein described camphor substitutes, being substances which act as solvents of nitrocellulose, or cellulose acetates, is illustrated 90 in the following examples.

Example I: 200 parts of the cellulose acetate herein above referred to, which is insoluble or difficultly soluble in chloroform but readily soluble in a mixture of chloroform and alcohol are dissolved by adding in a mixture of 200 parts of alcohol and 200 parts of dichlorethane or dichlormethane, together with any one or more of the camphor substitutes above referred to. The 95 solution thus obtained is employed for the 100 production of films or coatings or the like.

Example II: 100 parts of cellulose acetate, particularly the cellulose acetate above referred to, are dissolved in a heated mixture of equal volumes of alcohol and trichlorethylene, together with any one or more of the above mentioned camphor substitutes. The 110 solution in this example remains liquid when cold.

In the above examples one or more of the 115 camphor substitutes mentioned can be employed, together with any of the above mentioned solvents, in which the particular cellulose acetate employed, is soluble. Some of these camphor substitutes possess alone or mixed two or more together a dissolving power for these acetates of cellulose or cellulosic esters, which are insoluble in chloroform, but soluble in chloroform-alcohol. Some of these products or mixtures of 120 two or more also dissolve those acetates of cellulose which are soluble in chloroform. The non-inflammable celluloid masses thus 125

obtained, *i. e.*, solutions of cellulosic esters serve industrially as substitutes for celluloid and for the manufacture of objects, articles, products, etc., of every nature, such as films, 5 varnishes, coatings, artificial silk, artificial leather, etc.

What I claim is:—

1. A process of making a celluloid substitute which comprises dissolving a cellulose 10 ester of a fatty acid in a solvent including an etherified phenol.

2. A process of making a celluloid substitute which comprises dissolving a cellulose ester of a fatty acid in a solvent including 15 alcohol and an etherified phenol.

3. A process of making solutions for the manufacture of celluloid substitutes which comprises dissolving a cellulose acetate in a solvent including an etherified phenol.

20 4. A process for making solutions for the manufacture of celluloid substitutes which comprises dissolving a cellulose ester of a fatty acid in a solvent including alcohol,

chlorin derivatives of fatty hydrocarbons and an etherified phenol.

5. A celluloid substitute including a cellulose ester of a fatty acid and a solvent including an etherified phenol.

6. A celluloid substitute including a cellulose ester of a fatty acid and nitrocellulose 30 and a solvent including an etherified phenol.

7. A celluloid substitute including a cellulose acetate not readily soluble in tetrachloroethane, but readily soluble in alcohol-tetra-chlorethane mixture, and a solvent including 35 an etherified phenol.

In testimony whereof I have hereunto set my hand in the presence of two subscribing witnesses.

Paris, dated this 20th day of September, 40  
1911.

DR. HENRY DREYFUS.

Witnesses:

H. C. COXE,  
CAMILLE DREYFUS.